

## UNITED STATES PATENT OFFICE

2,240,447

## ROOFING AND THE LIKE

Richard A. Wilkins, Rome, N. Y., assignor to  
Revere Copper and Brass Incorporated, Rome,  
N. Y., a corporation of Maryland

No Drawing. Application October 30, 1940,  
Serial No. 363,515

3 Claims. (Cl. 108—13)

My invention relates to roofing and the like. Heretofore the material commonly employed for copper roofing, sheathing, and other exposed protective coverings for buildings has been thin sheets made by melting highly refined copper, casting the molten material into slabs, either hot or cold rolling the slabs into sheets of the desired thickness, and finally soft annealing the rolled sheets to a "dead soft" temper.

The copper for roofing has been refined in various ways, electrolytically refined copper, which commonly is 99.9% pure copper, being used almost exclusively during the past forty years. In refining copper for these purposes it has heretofore always been the practice of producers thereof to remove so far as possible all impurities so as to secure as pure a copper as possible. The known high resistance of pure copper generally to chemical corrosion, and the observed fact that impurities commonly found in rolled copper tend to make it less ductile in both the hot and cold rolled conditions, more difficult to produce by either hot or cold rolling, and commonly "cold short" in the sense that it tends to crack when bent or otherwise cold worked, have caused such pure copper heretofore to be considered the most satisfactory commercially available material for light weight metal roofing and the like.

However, it is a frequently observed fact that copper roofing, even when substantially 100% pure electrolytically refined copper, often fails in use, being subject to cracking sufficient to render it non-waterproof. Heretofore it was believed that these cracks were caused by mechanical fatigue resulting by reason of the cyclic stresses set up by alternate expansion and contraction of the copper sheets under varying temperature conditions. For this reason builders have resorted to expensive roof constructions, and various expensive expedients such as corrugating the roofing and the employment of elaborately designed expansion joints, and the use of heavy gauge copper in the attempt to relieve or reduce the effect on the roofing of these cyclic stresses and thereby eliminate so far as possible this form of failure. Although these attempts have been partially successful, the expense incidental thereto, and the many failures which actually have occurred in spite of these precautions, have seriously interfered in recent years with the general adoption of this otherwise very satisfactory roofing.

Prolonged investigations by applicant covering a period of years have demonstrated that the reason for the failure of copper roofing and the

like heretofore has not been correctly understood. This material, he has found, does not fail primarily by reason of the cyclic stresses to which it is subjected when in use, as heretofore believed, but, strangely enough, primarily by reason of a heretofore wholly unsuspected type of corrosion which occurs when this highly pure copper is exposed to an atmosphere contaminated by wind borne products of combustion of modern domestic and industrial fuel burning appliances and industrial atmospheres in general.

Applicant has found, that upon removing the patina and other accumulated corrosion products from copper roofing which has failed, the copper surface thus exposed is characteristically slightly pitted, instead of being in its smooth unpitted condition in which it originally left the rolling mill or the metal showing a uniform decrease in thickness over its whole surface due to corrosion.

His investigations indicate that these slight pits are caused by the formation on the copper, when exposed to a contaminated atmosphere, of a film of corrosion products which is characterized by a lack of adhesion to the copper, a lack of tenacity in respect to failure, and a tendency toward perviousness which allows the copper to be attacked locally rather than uniformly by the corrosive media and thereby result in the formation of sharply defined inwardly pointed pits in the nature of notches. Copper so attacked rapidly fails when subjected to the cyclic stresses hereinbefore referred to by reason of the natural tendency of the stresses to be concentrated in the metal below the bottoms of the notch-like pits. As a result of this concentration of the stresses the fatigue strength of the material is exceeded at the pits and the metal cracks.

Pure copper roofing as heretofore compounded applicant has found is comparatively sensitive to this "notch effect" when caused by a combination of chemical pitting and subjection to cyclic stresses. This sensitivity, it has been found, is very closely correlated to sensitivity to "work hardening" of the material when cold worked, each varying directly with the other. When pure copper roofing is cold worked it has been found that 50% of the hardness possible to be secured with any amount of cold working will be produced with as little as 5% cold working as, for example, reducing the thickness of pure copper roofing from 0.021 to 0.020 inch will increase its hardness to 50% of the maximum that could be effected by reducing its thickness to the maximum extent possible. This small amount of cold working will occur at the pits when pitted copper

roofing is subjected to the above mentioned cyclic stresses, which stresses may bend the material alternately back and forth, alternately stretch and compress it, or otherwise work it. On account of this, and the character of the notch-like pits, the resistance to cracking or other fatigue strength of the pure copper roofing, when subjected to cyclic stresses and to a contaminated atmosphere causing the pits, is reduced, it has been found, to as much as 20% of that of the original material as it left the mill.

Applicant has found that the above type of failure of copper roofing as constructed from thin sheets, commonly from about 0.003 to 0.03 inch in thickness, can be substantially entirely avoided by incorporating into the copper controlled amounts of arsenic, while otherwise maintaining the substantial purity of the copper by taking such precautions as will avoid the presence of certain deleterious constituents which might be entered into the copper with the arsenic or otherwise.

With the improved copper roofing it has been found that the surface of the copper, after the patina or other accumulated products of corrosion are removed, is in an unpitted condition, any corrosion which has occurred being uniformly distributed over its surface. Hence with the improved roofing there is no possibility of failure by "notch effect" as a result of a combination of chemical corrosion and subjection to cyclic stresses.

Further, the improved roofing as compared to prior copper roofing may, by proper control of the arsenic content, be made markedly less sensitive to notch effects occasioned by the presence of scratches, dents or other abrasions usually introduced during handling of the roofing or its installation. This results as a consequence of the presence of the arsenic, when in proper amount, rendering the roofing more immune to cracking when subjected to cyclic stresses.

It has been demonstrated by laboratory experiments and field tests that the presence of the proper amount of arsenic in the copper roofing produces on its surface a corrosion film which is tenacious, adherent, impervious and non-hygroscopic, the film being comparably as ductile as the copper base material itself, thus permitting the roofing to be repeatedly bent without rupture of the film or interruption of its adherence to the copper. Further because of these properties the film effectively protects the underlying base material from contaminated air and moisture, and thus effectively eliminates the possibility of the formation of the above mentioned pits.

This highly protective film, which forms in the matter of a few minutes or hours after exposure of the improved roofing, applicant believes is caused by an electro-chemical reaction. The film chemically is largely composed of arsenic compounds which are inherently more noble than either pure copper or compounds formed by the corrosion of pure copper when subjected to a contaminated atmosphere. Because of this characteristic of the film and its continuity and imperviousness it prevents the continued corrosion which occurs in pure copper roofing after initial corrosion by a contaminated atmosphere forms thereon a film of corrosion products, because with pure copper the film is loose, friable and incompletely adherent, and because of this is in effect less noble than pure copper. Furthermore this protective film formed on the improved roofing has the property of being essen-

tially self-healing in that if for any reason its continuity is locally interrupted it will substantially immediately reform and thus act to retard local corrosion at the interrupted regions which in a pure copper would continue to corrode at an accelerated rate resulting in formation of pits and as a consequence serious loss of fatigue strength of the roofing.

It will therefore be understood that arsenic is added to the roofing primarily for the purpose of increasing its corrosion resistance, for preventing it from pitting when subjected to atmospheric corrosion, and for decreasing its sensitivity to failure by "notch effect" under the cyclic stresses to which roofing is subjected.

Appreciable effects in the above respects will be observed with as little as about 0.02% arsenic. The maximum effect in respect to the primary purposes for which the arsenic is added is had with about 0.5% arsenic, with which amount the protective film will form in a practical sense substantially immediately on and be distributed continuously and uniformly over the exposed metal and thereby act effectively to prevent further corrosion of any kind. As the arsenic is increased above about 0.5% some effect in respect to increased resistance to corrosion and pitting is observed, an increase in the arsenic to 1% resulting in an increase of only about 10% in these resistances. However, as the arsenic is increased above 0.5% the high insensitivity to "notch effect" rapidly decreases, the roofing tending to become more sensitive to "work hardening" and as a result more sensitive to failure when subjected to cyclic stresses. Therefore an amount of arsenic in the neighborhood of 0.5% is preferably employed, say an amount within the range of 0.35 to 0.65%. For some purposes, say where the tendency to pit would be great on account of severe contamination of the atmosphere, larger amounts of arsenic may be employed, say up to 1 or 1.5%, which would cause the protective film to contain a larger percentage of arsenic compounds than in the case of a lower arsenic content of the roofing with the result that the film would be more resistant to the corrosive media. Such improvement however in the film and resistance of the roofing to corrosion would be gained at a slight sacrifice of the resistance to "notch effect," although in this latter respect the roofing with the higher amounts of arsenic would still be superior to pure copper roofing.

Applicant has found that best results ordinarily will be secured when the roofing does not contain impurities which tend to render it less malleable in the hot and cold conditions and thus tend to cause the hot or cold rolling or other working of the roofing during its fabrication to result in sub-microscopic surface cracks therein analogous in their effects to pits.

Among these deleterious substances are lead, bismuth, iron, nickel and sulphur, all of which tend to make the copper roofing either more difficult to produce or less resistant to the combined effects of cyclic stresses and corrosion. More than about 0.002% lead or 0.001% sulphur tends to make the material deleteriously less malleable in the hot condition. More than a trace of bismuth tends to make it deleteriously less malleable in both the hot and cold conditions. More than about 0.005% iron or nickel tends to make it more sensitive to "work hardening" and in consequence more sensitive to notch effects. Further, more than above these amounts of bismuth, sulphur, iron and nickel acting in-

dividually or in combination with each other causes arsenic-bearing copper roofing to approach the poor resistance of pure copper roofing to corrosion and its sensitivity to notch effects, and thereby act to destroy the beneficial effects of arsenic. The presence of such substances as cobalt, tin, silicon and zinc in substantial amounts had also best be avoided as they tend to increase the sensitivity of the copper roofing to "work hardening" and "notch effect." It thus will be understood, that in the sense the copper roofing does not contain deleterious substances or amounts thereof which substantially destroy the beneficial effects tended to be imparted by the arsenic, the balance of the alloy in respect to the arsenic is essentially copper.

In making the copper alloy roofing according to the invention the copper may be melted, and the arsenic added to the melt in the form of a copper-arsenic alloy, rich in arsenic. The molten metal may then be cast into slabs, which latter may be rolled into sheets of desired thickness by the usual mill process of rolling copper sheets. Finally the rolled sheets are annealed to the degree of softness that will best resist the cyclic stresses to which they are subjected when in use.

For convenience in terminology the article of manufacture according to the invention is termed "roofing," it being understood that as used in the appended claims such term includes various shingles, sheathings, valleys, and like protective

coverings for buildings, as well as what in a more limited sense is ordinarily termed "roofing." Also it will be understood that the roofing according to the invention comprises sheet copper presenting an extensive external roofing surface, and may in this sense consist of a backing having an exterior sheet of copper as well as consist wholly of sheet copper.

I claim:

- 10 1. Roofing comprising sheet copper presenting an extensive external roofing surface, the copper being alloyed with such amount of arsenic between 0.02 and 1.5% as will cause the formation on said surface when exposed to atmospheric corrosion of a self-healing, adherent, protective film composed predominantly of arsenic compounds, while rendering the sheet copper less sensitive to failure by reason of notch effect than sheet copper without the arsenic when subjected to the cyclic stresses caused by expansion and contraction of the roofing.
- 15 2. Roofing comprising sheet copper presenting an extensive external roofing surface, the copper being alloyed with approximately 0.02 to 1.5% arsenic, the balance of the alloy in respect to the arsenic being essentially copper.
- 20 3. Roofing comprising sheet copper presenting an extensive external roofing surface, the copper being alloyed with approximately 0.35 to 0.65% arsenic, the balance of the alloy in respect to the arsenic being essentially copper.

RICHARD A. WILKINS.